

Nov. 7, 1972

HIDEHISA YAMAGISHI ET AL  
PROCESS FOR PRODUCING MANGANESE DIOXIDE  
FOR DRY CELLS  
Filed Aug. 21, 1970

3,702,287

FIG. 1



FIG. 2



FIG. 3



FIG. 4



FIG. 5



## 1

3,702,287

### PROCESS FOR PRODUCING MANGANESE DIOXIDE FOR DRY CELLS

Hidehisa Yamagishi and Mizuo Tanaka, Kawasaki, Japan, assignors to Nippon Kokan Kabushiki Kaisha, Tokyo, Japan

Filed Aug. 21, 1970, Ser. No. 66,048

Claims priority, application Japan, Aug. 25, 1969,  
44/66,556

Int. Cl. B01k 1/00; C01b 15/04  
U.S. Cl. 204—83      6 Claims

#### ABSTRACT OF THE DISCLOSURE

Manganese dioxide is produced by direct current electrolysis of aqueous sulfuric acid solution of manganese sulfate under specified conditions.  $Mn^{3+}$  ions are produced and are hydrolyzed with the formation of  $MnO_2$ .

The present invention relates to a process for producing manganese dioxide by D.C. electrolysis of an aqueous sulfuric solution of manganese sulfate, wherein it comprises maintaining the anodic current density high, and also the concentration of sulfuric acid high, maintaining the temperature of electrolyte relatively high, so as to carry out hydrolysis of  $Mn^{3+}$  ion produced thereby, forming relatively coarse particles of  $MnO_2$  and filtering it thereafter, heating the  $MnO_2$  thus obtained in electrolyte, thus producing  $MnO_2$  simply, inexpensively and efficiently, which has an excellent property as a depolarizer for dry cells, and at the same time, to utilize the filtrate produced after the filtration of  $MnO_2$  for leaching manganese (as  $MnSO_4$ ) from suitable raw material.

Heretofore, it has been well known to obtain manganese dioxide as the depolarizer for dry cells by D.C. electrolysis of a manganese sulfate solution, which comprises producing manganese dioxide, and applying thereon a washing and other after-treatments. The process of the production is as follows.

The electrolysis is carried out by a process, with conditions including: composition of electrolyte by 20–150 g./liter of  $MnSO_4$  and 15–80 g./liter of  $H_2SO_4$ ; temperature of electrolysis, above room temperature (for example: 30–100° C.); current density, 1–2 a./dm.<sup>2</sup>; depositing manganese dioxide in lump form on the anode (usually graphite or lead, sometimes titanium), then stripping it off from the anode, and to obtain the product by subjecting the material with trituration or other after-treatments. Another process is disclosed in Japanese patent application No. 1,696/1966 (published on Feb. 2, 1966), that is, the electrolysis is carried out at conditions: the composition of electrolyte, 10–30 g./liter of  $Mn^{2+}$  and 100–350 g./liter of free  $H_2SO_4$ ; temperature, 10–30° C. (preferably 20° C. or below); current density, 35.5–59.2 a./dm.<sup>2</sup>; electrolytically oxidizing  $Mn^{2+}$  ions and hydrolyzing  $Mn^{3+}$  formed thereby, depositing granular  $MnO_2$ , filtering and washing the product. A process has been proposed to use, by recirculating, the waste liquid from electrolysis for leaching of ores. However, since the former process is a batch type electrolysis and the current density is low, the productivity is low. In the

## 2

latter process, the exothermic phenomenon is conspicuous because of the high current load, and it becomes necessary to dissipate the heat, so that a large capacity cooling device is required in order to maintain the specified temperature of 10–30° C. (preferably below 20° C.) especially under a weather condition as in Japan, especially in summer. Thus, the amount of production per unit electrolytic cell becomes small as it is limited by the cooling capacity, so that it is not economical. Moreover, the product  $MnO_2$  obtained by this process has a low purity and a large content of combined water, so that it has less favorable characteristics as a depolarizer for dry cells.

In the case where the manganese is leached as a sulfate from manganese-bearing containing ores, and when the raw material is in a form of oxides ( $Mn_3O_4$  or  $MnO$ ), it is necessary to add heat to effect solution to obtain a sufficient reaction rate.

Next, an oxidizing agent is added to the solution to remove impurities, especially metals (for example, Fe, etc.), contained in the raw material, to change  $Fe^{2+}$  into  $Fe^{3+}$ , then it is necessary to precipitate the metals of impurities as hydroxides, such as  $Fe(OH)_3$ , by filtration and separation in regulating the pH about 5. However, there were disadvantages that, when the solution is heated and regulated to have a pH of about 5,  $Mn^{3+}$  ions are hydrolyzed rapidly, producing a yellowish brown colloidal lump which is difficult to filter, and there is a loss of electrical energy required for oxidizing  $Mn^{2+}$  into  $Mn^{3+}$  ions, so that the current density is decreased.

The object of the present invention is to overcome and improve the above-mentioned disadvantages of conventional processes, and specifically, to deposit  $MnO_2$  in the electrolyte by selecting the above described electrolytic

conditions. Namely, the invention is to provide a process for obtaining manganese dioxide for dry cells comprising, selecting operational conditions as: composition of electrolyte  $Mn^{2+}$ , 10–40 g./liter; free  $H_2SO_4$ , 400–600 g./liter; temperature, 30–50° C.; anodic current density, 30–75 a./dm.<sup>2</sup>; anode being made of lead, lead alloy or lead oxide (for example, pure  $PbO_2$  produced by electrodeposition), electrolyzing by D.C. while agitating solution to oxidize  $Mn^{2+}$  so that 5–15 g./liter of  $Mn^{3+}$  is contained in the electrolyte, carrying out a hydrolyzing reaction gradually according to the following formula:



so as to produce  $MnO_2$  in the electrolyte, and to effect aftertreatments such as filtering, washing, drying, etc.

The further object of the present invention is to provide a process of producing efficiently manganese dioxide having an excellent discharge characteristic which comprises heating and agitating an electrolyte (containing  $Mn^{2+}$  and free  $H_2SO_4$  having said concentration, 5–15 g./liter of  $Mn^{3+}$  produced by the electrolysis and  $MnO_2$  produced by hydrolysis of  $Mn^{3+}$ ) taken out of the electrolytic cell at a temperature of about 50–100° C. for 0.5–4 hrs., to obtain the product after filtering, washing, and drying the  $MnO_2$ , or heating the electrolyte after filtering the produced  $MnO_2$  from said electrolyte so as to convert  $Mn^{3+}$  contained in the solution almost up to  $MnO_2$ , filtering it and adding  $MnO_2$  which has been filtered first to this electrolyte which contains almost no  $Mn^{3+}$  (contain-

ing 0.1-0.7 g./liter of  $Mn^{3+}$ ) by said heating and filtering, heating it while substantially returning  $MnO_2$  formed by heating of  $Mn^{3+}$  to the electrolytic cell, subjecting the product after-treatments such as filtering, washing, drying, etc.

Here, temperature is determined at 30-50° C., because it requires a large capacity of cooling device in order to maintain a temperature less than 30° C., taking the temperature rise due to exothermic effect at the electrolysis into consideration. Accordingly the yield per electrolytic cell is restricted, and when the temperature is above 50° C.,  $MnO_2$  is liable to adhere on the surface of the anode which prevents the formation of  $Mn^{3+}$  ions, leading to a sudden decrease in current efficiency, and at the same time, brown-colored, minute particles are produced which are not appropriate for depolarizer for dry cells. The reason for selecting the anodic current density at 30-75 a./dm.<sup>2</sup> is that, with the density below 30 a./dm.<sup>2</sup>, the productivity is low, and with the density more than 75 a./dm.<sup>2</sup>, the current conducting members are overheated due to heavy current load and that minute particles are produced which are not adequate for depolarizer for dry cells.

With a free  $H_2SO_4$  concentration below 400 g./liter,  $MnO_2$  is deposited at the anode when the temperature reaches to 30° C., and which decreases in the current efficiency, thus it is not satisfactory.

When  $MnO_2$  is heated in the electrolyte, the heating temperature is limited to 50-100° C. and the period is limited to 0.5-4 hours. This is because, with heating conditions with a temperature of below 50° C. and heating time below 0.5 hour, it is not possible to obtain an improvement in the purity of  $MnO_2$  due to oxidation of lower oxides, nor an improvement in the characteristics of the product as a depolarizer. While with a heating condition of a temperature above 100° C. and the heating time more than 4 hours, the oxidation of the lower oxides does not proceed in proportion to the increase in temperature and time, so that the improvement in the characteristic of the product as a depolarizer cannot be expected.

The invention will now be described referring to the drawings, in which:

FIG. 1 is a flow diagram showing the process for production of manganese dioxide according to the process of the present invention;

FIG. 2 is a graph showing the relation between the heating temperature when  $MnO_2$  is heated in the solution and the content of the combined water of  $MnO_2$ ;

FIG. 3 is a graph showing the relation of the heating temperature and purity of  $MnO_2$ ;

FIG. 4 is a graph showing the relation between the heating temperature and the content of lower oxide in  $MnO_2$ ; and

FIG. 5 is a graph showing the relation between the heating time and the content of lower oxide in  $MnO_2$ .

In the drawings the broken lines show the course of the oiliquid, slurry, etc.

raw material and  $MnO_2$ , while the full lines show the

Referring to FIG. 1, the raw material and aqueous sulfuric solution of manganese sulfate to be used as a circulating acid are introduced in a leaching tank 1, to leach manganese component from the raw material. The manganese sulfate solution is supplied continuously to the electrolytic cell 2, and the D.C. electrolysis is carried out under agitation at a specified temperature.

$Mn^{2+}$  is oxidized electrolytically to  $Mn^{3+}$ , and is hydrolyzed gradually, and  $MnO_2$  is deposited in the electrolyte.

Slurry containing  $MnO_2$  and  $Mn^{3+}$  ions is continuously discharged from the electrolytic cell 2, and the slurry is filtered by a filter to separate it into  $MnO_2$  and the filtrate. The filtrate contains  $Mn^{3+}$  at high concentration together with  $H_2SO_4$  and  $Mn^{2+}$ , the major part of which

are returned to the cell 2, and a portion thereof is heated in a heat-treatment tank 4, hydrolyzing  $Mn^{3+}$  to produce  $MnO_2$ , filtering it in a filter 5, returning the produced  $MnO_2$  to the electrolytic cell 2, which is used as seed, and the filtrate is passed to the heat-treatment tank 6. In some cases, the filtrate of the filter 3 is passed directly to the heat-treatment tank 6.  $MnO_2$  obtained on the filter 3 is passed to the heat-treatment tank 6 and (the solution containing the filtrate from the filter 5, which contains  $H_2SO_4$ ,  $Mn^{2+}$  and whose  $Mn^{3+}$  concentration is decreased to about the equilibrium state by heating), is heated together with the filtrate from the filter 3 or after which filtering it by a filter 7 and separate it into  $MnO_2$  and the filtrate.

$MnO_2$  is subjected to treatments such as neutralizing and washing 8, drying 9, etc., and is made into a product. The filtrate from 7 contains free sulfuric acid,  $Mn^{2+}$ , and low concentration  $Mn^{3+}$ , but it is returned to the leaching tank 1, and is used for leaching manganese from the raw material as a circulating acid.

Considered from the thermo-economical point of view, the heat required for heating 4 of the filtrate containing high concentration  $Mn^{3+}$  after separation 3 of  $MnO_2$  discharged from the electrolytic cell 2 can be utilized for heating of  $MnO_2$  in the following heat-treatment tank 6, and the heat required for heating the latter may be utilized effectively for leaching manganese portion from the raw material in the next leaching tank 1.

FIG. 2 is a graph showing a relation between the heating temperature and the content of combined water when  $MnO_2$  is heated in electrolyte. When the content of the combined water is decreased by heating it at a temperature more than 100° C. in air for a long time, the performance is deteriorated as a depolarizer for dry cells, but when the content of the combined water is decreased by a heating in a solution as shown in FIG. 2, the depolarizing capacity is remarkably improved. FIG. 3 is a graph showing a relation between the heating temperature and the purity of  $MnO_2$ , and it shows that the purity is increased as the heating temperature is increased. FIG. 4 is a graph showing a relation between the heating temperature and the content of lower oxide in  $MnO_2$ , and FIG. 5 is a graph showing a relation between the heating time and the quantity of lower oxide in  $MnO_2$ . They show that the content of the lower oxide is decreased as heating temperature is increased, as well as heating time is increased.

Some examples are given in the following:

## EXAMPLE I

### (A) Electrolysis

Electrolytic cell: 4 liters

Electrode:

Anode: Pure  $PbO_2$  formed by electro-deposition

Cathode: Graphite

Distance between electrodes: 9 mm.

Composition of electrolyte:

Concentration of free sulfuric acid: 400 g./liter

Concentration of  $Mn^{2+}$ : 20 g./liter

Temperature: 37° C.

Current density: 45 a./dm.<sup>2</sup>

Mean bath voltage: 3.7 v.

Raw material:  $MnSO_4$  solution containing 120 g./liter as  $Mn^{2+}$

Quantity of raw material supplied: 200 ml./hr., continuous feeding

### (B) Heating after electrolysis

Heating temperature: 95° C.

Heating time: 2 hours

Electrolyte used for heating contained 400 g./liter of  $H_2SO_4$ , 20 g./liter of  $Mn^{2+}$  and 0.3 g./liter of  $Mn^{3+}$

(C) Current efficiency and composition of MnO<sub>2</sub> produced

Current efficiency: 76.0%, 6 hours of electrolysis  
Product:

Total Mn: 58.6%

MnO<sub>2</sub>: 87.9%

Combined water: 7.0%

Pb: 0.009%

Crystal structure:  $\gamma$ -MnO<sub>2</sub>

## EXAMPLE II

## (A) Electrolysis

Electrolytic cell, electrodes and the distance between electrodes are the same as in Example I.

Composition of electrolyte:

Concentration of free sulfuric acid: 500 g./liter

Concentration of Mn<sup>2+</sup>: 16 g./liter

Temperature: 45° C.

Current density: 60 a./dm.<sup>2</sup>

Mean bath voltage: 4.3 v.

Material: MnSO<sub>4</sub> solution containing 110 g./liter as Mn<sup>2+</sup>, obtained by leaching MnCO<sub>3</sub>

Quantity of raw material supplied: 240 ml./hr. continuous feeding

## (B) Heating after electrolysis

Heating temperature: 70° C.

Heating time: 3 hours

Electrolyte used for heating contained 500 g./liter of H<sub>2</sub>SO<sub>4</sub>, 16 g./liter of Mn<sup>2+</sup> and 9.5 g./liter of Mn<sup>3+</sup>(C) Current efficiency and composition of MnO<sub>2</sub> produced

Current efficiency: 71.2%, 24 hrs. of electrolysis

Product:

Total Mn: 58.0%

MnO<sub>2</sub>: 86.4%

Combined water: 9.8%

Crystal structure:  $\gamma$ -MnO<sub>2</sub> and a small amount of  $\alpha$ -MnO<sub>2</sub>

## EXAMPLE III

## (A) Electrolysis

Same cell as in Example I

Electrodes: Both anode and cathode are made of Pb

Distance between electrodes: 14 mm.

Composition of electrolyte, the same as in Example I

Temperature: 40° C.

Current density: 50 a./dm.<sup>2</sup>

Mean bath voltage: 3.9 v.

Material: MnSO<sub>4</sub> solution containing 100 g./liter as Mn<sup>2+</sup>, obtained by leaching MnO

Quantity of raw material supplied: 210 ml./hr., continuous feeding

## (B) Heating after electrolysis

Heating temperature: 80° C.

Heating time: 1.5 hrs.

Electrolyte used for heating is the same as Example I

(C) Current efficiency and composition of MnO<sub>2</sub> produced

Current efficiency: 73.5%, 48 hrs. of electrolysis

Product:

Total Mn: 58.3%

MnO<sub>2</sub>: 87.0%

Combined water: 7.5%

Crystal structure:  $\gamma$ -MnO<sub>2</sub> and a small quantity of  $\alpha$ -MnO<sub>2</sub>6  
EXAMPLE IV

As the result of discharge performance test by 10 ohm continuous discharge based on JIS K 1467-1965, it was found that MnO<sub>2</sub> produced by the process according to the present invention, has "duration of closed-circuit at a voltage of more than 1.0 v." is increased about 15-20% as compared with the conventional products, and that it has remarkably excellent characteristics as depolarizer.

## 10 TABLE I.—DISCHARGE PERFORMANCE

|                                                                      |  | Minutes <sup>1</sup> |
|----------------------------------------------------------------------|--|----------------------|
| Commercial electrolytic MnO <sub>2</sub>                             |  | 215                  |
| MnO <sub>2</sub> produced by Japanese patent publication No. 1696/66 |  | 200                  |

15 MnO<sub>2</sub> produced according to the process of the present invention

<sup>1</sup> Duration of closed-circuit at a voltage of more than 1.0 v.

20 As stated above, the effect or advantages of the present invention shown in the examples can be summarized as follows:

25 Since the temperature selected is high such as 30-50° C., no cooling device is needed for electrolyte, and it is easy to maintain the temperature constant. By heating MnO<sub>2</sub>, produced by the electrolysis in the electrolyte having said composition, there were obtained a decrease in the quantity of combined water, increase in purity of MnO<sub>2</sub>, decrease in lower oxide as shown in FIGS. 2-5;

30 "the duration of closed-circuit at a voltage of more than 1.0 v." is increased about 15-20% as compared with the conventional products, thus MnO<sub>2</sub> having remarkably excellent characteristics as a depolarizer was obtained. Moreover, by this heating, Mn<sup>3+</sup> ions contained in the

35 solution are decomposed and deposited as MnO<sub>2</sub>, and through which Mn<sup>3+</sup> ions remaining in the solution can be lowered up to the equilibrium concentration, so that even when the solution is used for leaching of manganese from the raw material, the loss of electric energy

40 due to hydrolysis of Mn<sup>3+</sup> ions, and therefore the decrease in current efficiency can be restricted to a minimum. Also, by adopting a series of procedures shown in FIG. 1, the heat required for heating the electrolyte, containing high concentration Mn<sup>3+</sup> after separation of

45 MnO<sub>2</sub> discharged from electrolytic cell, can be utilized for heating of MnO<sub>2</sub> in the following electrolyte, and the heat required for heating MnO<sub>2</sub> in said electrolyte can be utilized effectively for leaching manganese from the raw material, respectively.

50 What is claimed is:

1. In an electrolytic process for producing manganese dioxide suitable for dry cells wherein direct current electrolysis is employed, the improvement which comprises conducting said electrolysis with an electrolyte containing a concentration of from 10 to 40 grams per liter of Mn<sup>2+</sup> ion and from 400 to 600 grams per liter of free H<sub>2</sub>SO<sub>4</sub>, a temperature of from 330° C. to 50° C., and an anodic current density of from 30 to 75 a./dm.<sup>2</sup>, to oxidize Mn<sup>2+</sup> therein to Mn<sup>3+</sup>, and hydrolyzing the resulting

60 product containing Mn<sup>3+</sup> to form MnO<sub>2</sub> in the electrolyte.

2. Process of claim 1, wherein said resulting product contains from 5 to 15 grams per liter of Mn<sup>3+</sup>.

3. Process of claim 1, wherein said electrolyte containing MnO<sub>2</sub> is heated at a temperature of from 50° C. to 100° C. for from 0.5 hour to 4 hours.

4. Process of claim 2, wherein said electrolyte containing MnO<sub>2</sub> is heated at a temperature of from 50° C. to 100° C. for from 0.5 hour to 1 hour.

5. Process of claim 1, wherein MnO<sub>2</sub> is separated from the electrolyte containing MnO<sub>2</sub> and is returned to said electrolysis.

6. Process of claim 1, wherein MnO<sub>2</sub> (1) is filtered from the electrolyte containing MnO<sub>2</sub>; the resulting filtrate is heated and fine crystals of MnO<sub>2</sub> (2) are filtered therefrom and are returned to said electrolysis; and

$\text{MnO}_2$  (1) is heated at a temperature of from 50° C. to 100° C. for from 0.5 hour to 4 hours in the filtrate obtained by filtration of  $\text{MnO}_2$  (2).

**References Cited**  
**UNITED STATES PATENTS**

3,065,155 11/1962 Welsh 204—83  
1,874,827 8/1932 Storey 204—83

2,500,039 3/1960 Magoffin et al. 204—83  
3,533,924 10/1970 Ve 204—67

JOHN H. MACK, Primary Examiner  
5 D. R. VALENTINE, Assistant Examiner

**U.S. CL. X.R.**